# EUROPEAN PATENT SPECIFICATION

(11) **EP 0 185 806 B1**
(45) Date of publication and mention of the grant of the patent: **09.03.1988**
(21) Application number: 84308470.8
(22) Date of filing: 06.12.1984
(51) Int. Cl.: D02G 3/44, D02G 3/16

(54) **Supported antistatic yarn, products incorporating same, and method for its production**
Antistatisches Garn, solch ein Garn beinhaltende Textilerzeugnisse und Verfahren zu seiner Herstellung
Fil antistatique, produits manufacturés comprenant un tel fil, et procédé de fabrication

(43) Date of publication of application: 02.07.1986
(73) Proprietor: BADISCHE CORPORATION, Williamsburg Virginia 23185 (US)
(72) Inventor: Gusack, James Andrew, Williamsburg Virginia 23185 (US); Smith, Thomas Edward, Virgina 23185 (US)
(74) Representative: Gore, Peter Manson

(56) References cited:
- DE-A- 2 106 784
- DE-A- 3 019 151
- FR-A- 2 060 679
- FR-A- 2 193 888
- US-A- 3 590 570
- US-A- 3 969 559
- US-A- 4 232 082

## Description

The present invention relates to supported, antistatic yarns, a process for making them and to products incorporating such yarns.

Antistatic yarns have been in use for some time and are incorporated in fabrics and carpets to reduce the build up of electrostatic charges thereon. Such antistatic yarns comprise one or more conductive strands together with one or more support strands. The support strands have been utilized to improve the performance with respect to beaming, knitting and weaving of such conductive strands. Conductive strands which are particularly useful in forming antistatic yarns are described in U.S. Patents 4,255,487 and 3,823,035 which disclose a method of making a conductive material by a process of suffusing conductive carbon black particles into a polymeric substrate.

Such antistatic yarns have previously been formed by twisting conductive strands with strengthening support strands to form a yarn. Such twisted antistatic ropes and yarns are described in U.S. Patents 3,206,923 and 3,291,897.

Whilst such twisted antistatic yarns provide improved performance over conductive strands in such operations as warping, weaving and knitting, it is frequently desirable to use twistless yarns in the production of antistatic products. It is one object of the present invention to provide twistless or substantially twistless antistatic yarns which nevertheless provide the desired improved performance in such process operations.

The production of supported conductive strands in the form of antistatic yarn involves an additional process step which adds to the cost of producing the final products produced by such downstream process operations. It is a further object of the present invention to provide an improved method in which the formation of a supported conductive strand in the form of an antistatic yarn is concurrently effected with the production of the conductive strand itself.

The antistatic yarns of the present invention are produced using a solvent bonding technique. A number of solvent bonding techniques have been proposed in the production of coherent products from stable fibre materials.

Thus, a process of solvent bonding has been proposed to bond staple fibres together to form a non-woven fabric. U.S. Patent No. 3,647,591 discloses such a process of making a non-woven fabric from a blend of staple fibres. In this patent a non-woven fabric containing a blend of staple fibres is contacted by an acid which softens only a specific type of fibre in the blend after which the blend is compressed to bond the fibres together.

The production of a twistless staple fibre yarn from a staple fibre material and a continuous filament yarn by a solvent bonding technique is described in U.S. Patent No. 3,945,186. This patent proposed a solution to the problem arising in addition of a continuous filament yarn to staple fibre which rendered it impossible to draft the mixed fibre ribbon thus produced. The selection proposed was to use a continuous filament yarn which could be brought into a plastic state by the action of an applied solvent prior to drafting so that the drafting of the mixed fibre yarn amounted to drafting of the staple fibre component of the mixed fibre yarn, the filamentary element also providing the means of bonding the staple fibre component.

U.S. 4,107,914 discloses a process of solvent bonding a sliver or roving of staple fibre into a twistless or substantially twistless yarn. The process requires a roving of staple fibres to be wetted with a mixture of a latent solvent and a more volatile liquid. The roving is then drafted, fibre twisted and brought into contact with a heated surface which first evaporates the volatile liquid and then activates the latent solvent which dissolves only a surface layer of staple fibres forming a substantial proportion of the sliver or roving and so bonds the staple fibres altogether, and thereafter evaporates the latent solvent from the yarn.

The solvent bonding methods in the prior art, as exemplified by the above mentioned U.S. Patents have been principally concerned with effecting bonding of staple fibres to form a strand which is then used as a component of a yarn, and in doing so have taken advantage of the well established wet drafting methods of producing such strands from slivers or rovings of staple fibres. The conductive strands which concern the present invention are already continuous and coherent as also are the support strands used in conjunction with such conductive strands to form antistatic yarns. The conventional methods of twisting and plaiting were therefor obvious expedients to use in the production of antistatic yarns and ropes from such already cohesive structures, especially as such conductive and support strands are composed of continuous filaments. The application of solvent bonding techniques previously known for staple fibre to the production of antistatic yarns was not an obvious expedient since such method would be expected on the one hand to provide yarns, especially when composed of continuous filaments having too little flexibility or if flexibility were sufficient to be insufficiently cohesive to withstand the further processes such as warping, weaving and knitting.

It has now been surprisingly found that when conductive strands are intermittently solvent bonded along their length to support strands, especially continuous filament support strands, the resulting antistatic yarn exhibits all the advantageous properties of the hitherto known twisted yarns in subsequent processing steps such as warping, weaving and knitting and can even possess superior properties to such twisted yarns.

According to the present invention there is provided an antistatic yarn comprising at least one conductive strand composed of synthetic plastics material, said conductive strand having finely divided electrically conductive material suffused thereinto, and at least one support strand composed of synthetic plastics material, characterised in that said conductive strand is intermittently solvent bonded along its length to said at least one support strand.

Preferably, the yarn comprises a plurality of support strands, said conductive strand being intermittently bonded along its length to more than one of said support strands.

The synthetic plastics material is preferably a polyamide, most preferably a polycaprolactane. The preferred finely divided electrically conductive material is carbon black, although any other equivalent material could be used. Preferably both the conductive strands and support strands are continuous filaments, the support strand most preferably being an interlaced yarn.

The antistatic yarn of the present invention finds use in the production of composite yarns composed of the antistatic yarn of the present invention interlaced into a carpet yarn. The present invention also encompasses carpets comprising the antistatic yarn of the invention.

The present invention also provides a method of producing an antistatic yarn which comprises suffusing a finely divided electrically conductive material into a strand composed of a synthetic plastics material to form a conductive strand by applying to the travelling strand a dispersion of said finely divided material in a liquid which is a solvent for synthetic plastics material of both the strand which is to become the conductive strand and the support strand, but does not dissolve or react with the said finely divided material, characterised in that the support strand or strands are brought into generally side-by-side relationship with the potentially conductive strand before a substantial amount of the solvent carried by the potentially conductive strand has evaporated therefrom and allowing said potentially conductive strand to contact said support strand or strands at intermittent points along the length thereof, the potentially conductive strand being allowed to contact only the support strand or strands and the atmosphere until the liquid has substantially evaporated from the potentially conductive strand and in that the evaporation of liquid being effected by passing the potentially conductive strand and the support strand or strands in generally side-by-side relationship and in contact at intermittent points along their length through an evaporation zone maintained at an elevated temperature whereby to effect intermittent solvent bonding of the conductive strand to the support strand or strands along the length thereof.

The Applicants have found that by bringing a moving support strand or strands into generally side-by-side relationship with a conductive or potentially conductive strand moving at the same speed, said conductive strand or said supportive strand or strands having provided on the surface thereof a solvent for the synthetic plastics material of both the conductive and support strands, surprisingly the conductive or potentially conductive strand will intermittently touch the support strand or strands at points along their length and form intermittent solvent bonded points or small areas and that subsequent evaporation of the solvent results in a coherent yarn without utilizing means to press the strands together. The strands must, of course, be brought into generally side-by-side relationship before any substantial amount of the provided solvent has evaporated so that the solvent action on the surfaces at the points of contact can cause solvent bonding to be effected.

At the point where the conductive or potentially conductive strand and the support strands first come into side-by-side relationship they should be no more than 3mm apart and most preferably should touch at this point.

In a preferred embodiment, the invention provides a method of forming an antistatic yarn which comprises suffusing a finely divided electrically conductive material into a strand composed of synthetic plastics material to form a conductive or potentially conductive strand and combining said conductive or potentially conductive strand with at least one support strand composed of synthetic plastics material to form a coherent yarn, characterised by providing a solvent for the synthetic plastics material of both the conductive or potentially conductive strand and the at least one support strand on the surface of the conductive or potentially conductive strand, bringing the conductive strand and the at least one support strand into generally side-by-side relationship and travelling at the same speed and in the same direction before a substantial amount of the provided solvent has evaporated, allowing said strands to touch each other at intermittent points along their length, whereby to effect intermittent solvent bonding of the at least one support strand with the conductive strand along the length thereof and effecting evaporation of the provided solvent to form a coherent antistatic yarn.

The suffusing of the finely divided electrically conductive material into the strand of synthetic plastics material may be effected in known manner by applying to the travelling strand a dispersion of the finely divided material in a liquid which is a solvent for the synthetic plastics material to form a potentially conductive strand and evaporating the solvent to form a conductive strand. In the most preferred method of the present invention, the said liquid is also a solvent for the synthetic plastics material of the support strands and the support strands are brought into generally side-by-side relationship with the potentially conductive strand before a substantial amount of the liquid has evaporated from the potentially conductive strand.

Contact of the solvent bearing strand and of the intermittently solvent bonded conductive or potentially conductive strand and the support strands with any other object or surface should be avoided before the solvent or in the case of the most preferred method, the liquid of the dispersion has evaporated. If such contact does occur it will result in accumulation of excessive solvent or liquid dispersion on such object or surface. The accumulation of excess solvent on such a surface could cause breaks to occur in the strands and in the most preferred method, if such accumulation (e.g. of liquid dispersion) is dislodged onto the strands, will cause a serious yarn and/or package defect. In the most preferred method therefore, it is especially desirable to avoid such contact and the potentially conductive strand should only be allowed to contact the support strand or strands and the atmosphere before the liquid has evaporated.

. The support strands and the conductive or potentially conductive strands are preferably brought into generally side-by-side relationship by passing the non-solvent bearing strand or strands over a guide such as a guide bar disposed adjacent but not touching, the moving solvent or liquid dispersion carrying strand so that the non-solvent-bearing strand or strands change direction to run generally parallel with the solvent or liquid dispersion bearing strand. Alternatively, but less preferably the conductive or potentially conductive and the support strands can be brought into generally side-by-side relationship by passing the solvent or liquid dispersion carrying strand through a hollow supply means (such as a pirn) for the non-solvent-bearing strand or strands and then passing both types of strand through a balloon guide, the solvent or liquid dispersion bearing strand passing through the centre of the balloon guide, but the non-solvent-bearing strands being in constant contact with the inside surface of the balloon guide, which arrangement has the effect of cabling the non-solvent-bearing strand or strands around the solvent bearing strand.

In the most preferred embodiment, the present invention provides a method in which the finely divided electrically conductive material is suffused into a strand of synthetic plastics material to produce a potentially conductive strand by applying to the travelling strand a dispersion of said finely divided material in a liquid which is a solvent for synthetic plastics material of both the strand which is to become the conductive strand and the support strands, but does not dissolve or react with said finely divided material, characterised in that the support strand or strands are brought into generally side-by-side relationship with the potentially conductive strand before a substantial amount of the liquid carried by the potentially conductive strand has evaporated therefrom and allowing said conductive strand to contact said potentially support strand or strands at intermittent points along the length thereof, the potentially conductive strand being allowed to contact only the support strand or strands and the atmosphere until the liquid has substantially evaporated from the potentially conductive strand whereby to effect intermittent solvent bonding of the conductive strand to the support strand or strands along the length thereof.

Preferably the evaporation of solvent, e.g. liquid of the liquid dispersion is effected by passing the potentially conductive strand and the support strand or strands in generally side-by-side relationship and in contact at intermittent points along their length through an evaporation zone maintained at an elevated temperature.

Most preferably, air at an elevated temperature is passed through the evaporation zone in countercurrent to the direction of travel of the potentially conductive and the support strands.

The solvent is selected according to the nature of the synthetic plastics materials. Thus, in the case of a polyamide, especially a caprolactam, the solvent is preferably formic acid.

The invention will now be further described by way of examples, with reference to the accompanying drawings, in which:-
Figure 1 is a schematic representation of the most preferred embodiment of the present invention;
Figure 2 is a schematic representation of an alternative process of carrying out the present invention;
Figure 3 is a partial enlarged longitudinal view of the product of the present invention;
Figure 4 is an enlarged view of a small portion of Figure 3; and
Figure 5 is a cross sectional view of the product of the present invention, Figure 5 being taken through line C-C of Figure 4.

Figure 1 is a schematic representation of the most preferred process for carrying out the present invention. A first pirn 1 having a first strand 2 wound thereon supplies a strand 2 to a conductive mix applicator 3. The strand 2 is most preferably a nylon-6 monofilamentary strand. The conductive mix applicator 3, shown schematically, is comprised of a reservoir (which contains a conductive mix), the reservoir having an inlet orifice and an outlet orifice through which the strand enters and exits the reservoir. Both orifices are sized slightly larger than the strand diameter. The strand exits the reservoir with a controlled amount of mix thereon. The mix is most preferably formic acid having nylon 6 polymer dissolved therein and conductive carbon black particles dispersed therein. The strand is pulled off of the first pirn 1 by a pair of rollers 4, the surface speed of each roller 4 being set at approximately 700 metres per minute. Once the first strand 2 emerges from the applicator 3, the first strand 2 travels into an evaporation tube 5. As the first strand, having mix thereon, approaches the entrance to the evaporation tube 5, a second strand 6 is brought into generally side-by-side relationship with the first strand 2, the second strand 6 most preferably being a nylon-6 multifilament strand, the second strand 6 being supplied from a second pirn 7. It should be noted that the second strand 6 is most preferably directed through a balloon guide 9 in order to confine the downstream motion of the second strand 6. The second strand 6 is brought into generally side-by-side relationship with the first strand 2 by placing a guide 8 above the entrance to the evaporation tube 5. The guide 8 serves as a contact point for the second strand 6, this contact point allowing the second strand 6 to change directions so that immediately downstream of the guide 8, the direction or travel of the second strand 6 and the first strand 2 is generally parallel. The speed of both strands 2 and 6 is controlled by the rollers 4. Both strands 2 and 6 travel at the same speed. The second strand 6 is threaded over the guide 8 so that the second strand 6 is between the guide 8 and the first strand 2, the guide being positioned so that there is a distance ranging from 0 mm to 3 mm between the first strand 2 and the second strand 6 at the point at which the second strand 6 contacts the guide 2. Most preferably the first strand contacts the second strand at the guide (i.e. the most preferred distance is 0 mm). However, it is also preferred that the path of travel of the first strand is substantially undeflected (unchanged) by the guide and the support strand. The first strand 2 and the second strand 6 travel into the evaporation tube in close proximity to one another, and it has been observed that the two strands 2 and 6 tend to "jump together" slightly downstream of the guide 8 when a distance no greater than 3 mm is maintained between the strands 2 and 6 at the guide 8. Most preferably the second strand 6 is an interlaced yarn.

Once the strands 6 and 2 enter the evaporation tube, the strands are subjected to a countercurrent (about 600 metres per minute) of hot air (most preferably 150°C), the hot air entering the evaporation tube at an inlet port 15 and exiting the evaporation tube at an exhaust port 10. The "break" 11 indicated in the figure is included in order to reveal the fact that the evaporation tube must be relatively long compared to the remainder of the process. Most preferably the distance from the first pirn 1 to the evaporation tube entrance is about 1 metre, while the length of the evaporation tube 5 is about 10 metres, and the distance from the evaporation tube exit to a yarn take-up pirn 12 is about 2 metres.

After the strands 2 and 6 are brought into generally side-by-side relationship at the guide 8, the mix applied to the first strand 2 contacts and spreads into the second strand 6 at points at which the first strand 2 contacts the second strand 6. As the strands 2 and 6, now together, travel through the evaporation tube, the mix suffuses into both yarns 2 and 6 and causes intermittent solvent bonding to occur at the contact points. Thus, upon emerging from the downstream end of the evaporation tube 5, a supported antistatic yarn 13 has been formed by the solvent-bonding occurring between the two strands 2 and 6 entering the evaporation tube 5. After emerging from the downstream end of the evaporation tube 5, the yarn 13 is directed around the rollers 4 which control the speed of the yarn, following which the yarn 13 is directed through a pigtail guide 14, following which the yarn is wound up onto the take-up pirn 12, the yarn 13 together with the take up pirn 12 forming a package of supported antistatic yarn.

Figure 2 is a schematic of an alternative process of the invention. The process illustrated in Figure 1 is used to make what may be termed a "simple side-by-side" supported antistatic yarn. However, in Figure 2 the second pirn 7 has the first strand 2 running longitudinally therethrough, the pirn 7 being hollow. The first strand 2 is directed through the mix applicator 3 before it enters the second pirn 7, and the first strand is directed through the centre of a balloon guide 8A after emerging from the second pirn 7. The second strand 6 is taken off the second pirn 7 and is also directed through the balloon guide 8A. The first strand 2 is aligned so that it travels through the centre of the guide 8A, while the second strand constantly remains on the inside surface of the balloon guide. Thus, in bringing the strand 2 and the strand 6 into generally side-by-side relationship, the process illustrated in figure 2 "cables" the support strand 6 around the antistatic strand 2. The process illustrated in figure 2 results in a "cabled supported antistatic yarn". The balloon guide 8A most preferably has a 4 mm wide inside diameter. This guide 8A is designated as being different from the guide 8 in Figure 1. The alternative process illustrated in Figure 2 requires a balloon guide, whereas the preferred process illustrated in Figure 1 may use, in addition to a balloon guide, any other guide which will hold the second strand 6 at the desired point alongside the path of the first strand 2. Aside from the description above, the alternative pro= cess illustrated in Figure 2 is no different from the preferred process illustrated in Figure 1. The process of Figure 1 is preferred for several reasons, including easier stringup and the convenience of using transfer tails on the second strand 6, this convenience enabling a "non-stop" process not possible with the embodiment shown in Figure 2.

Figure 3 is a partial enlarged view of the product of the present invention. The supported antistatic yarn 13 is shown in part, i.e. several nonconductive support strands are not shown for the sake of simplicity. Aconductive monofilamentstrand 31 is shown in combination with three nonconductive support strands 34. At two separate solvent-bonded points 32, the conductive strand has been solvent bonded to a nonconductive support strand 34.

Figure 4 shows an enlarged close-up view of one of the solvent bonds 32 shown in Figure 3. As can easily be seen in Figure 4, at the solvent-bonded point 32 the mix on the conductive strand 31 has spread onto the nonconductive support strand 34 to which the conductive strand 31 has solvent-bonded.

Figure 5 is a cross sectional view of the strands shown in Figure 4, the cross sectional view being taken through section C-C shown in Figure 4. Figure 5 shows the conductive strand 31 having an outer "coated" region 36 and an inner "suffused" region 35. The conductive strand 31 is solvent bonded to the support (nonconductive) strand 34, with the supporting strand 34 having an outer "coated" region 38 partially around and an inner. "suffused" region 37 also partially around. An interface region 39 is believed to exist between the conductive strand 31 and the nonconductive support strand 34. The interface region 39 is furthermore believed to resemble the outer "coated" regions 38 and 36.

In the most preferred embodiment of process of the present invention, the support strand is brought into general side-by-side relationship and intermittent contact with a conductive strand, e.g. a filamentary substrate both after the conductive strand has been coated with a conductive solvent-containing mix, and before the solvent has substantially evaporated from the mix. Thus the support strand is brought into general side-by-side relationship (i.e. ^{<_} 3mm) from the web conductive support at the guide 8 so that the two strands will "jump together" in time for an adequate frequency of solvent-bonded "weld points" to occur. In any event in order to avoid the risk of packing defects it is imperative that the conductive strand, once wet with the mix, contacts only the support strand and the atmosphere, or the mix will accumulate on any contact point and eventually will be picked up and carried by the conductive strand or the support strand. Any sizeable accumulation (i.e. a lump) of mix will probably contain so much solvent that it will fail to dry in the evaporation tube and will fuse windings of yarn together on the package, ruining the remainder of the package for downstream processing operations.

### Example

A conductive mix applicator was constructed from a first pipe having a length of55 mm and an i.d. of 10 mm. The first pipe was vertically oriented and securely mounted. From the side, a second pipe was connected to the midpoint of the first pipe. The second pipe had a shutoff valve thereon a short way back from the intersection of the second pipe with the first pipe. The shutoff valve was closed. The second pipe was connected to a pressurized source of conductive mix. Two jewelled bearings (synthetic sapphire watch bearings) were obtained from A. M. Gatti, Inc., 524 Tindall Avenue, Trenton, N.J. Each jewelled bearing had an outside diameter of 1.5 mm and a centrally located orifice having a diameter of 75 microns, and each bearing had a thickness of 0.5 millimetres. The bearings were swaged into stainless steel discs which had a diameter of 13 mm and a thickness of 1 millimetre. Each disc had a through hole which was centered and was 1.3 mm in diameter, the through hole having a counterbore 1.6 mm in diameter and 0.5 mm deep. The bearings were swaged into the counterbores. After both of the bearings were swaged into the counterbores, the discs were clamped onto the ends of the first pipe (i.e. each disc/bearing combination formed a "cap" on the ends of the first pipe). The bearings were about 55 mm apart. The clamping was performed so that watertight seals were formed betwen the pipe and the caps. The combination of the bearings, the discs, and the first pipe constitutes the conductive mix applicator.

A 20 denier polycaprolactam monofilamentary strand, having a diameter of 50 microns, was supplied from a first pirn mounted above the mix applicator. The cap on the upper end of the first pipe was removed, and the monofilament strand was threaded through the 75 micron orifice by hand. Several centimetres (about 0.254 metres) of monofilament strand were pulled through the orifice. The bottom cap was removed from the pipe and the upper cap was held close to the upper end of the first pipe while a slight vacuum was applied to the bottom of the first pipe. The airflow created by the vacuum caused the 0.254 metres of monofilament strand to be directed through the first pipe. The upper cap was then reclamped, with the monofilament strand threaded through both the upper cap (i.e. bearing) and the first pipe. The monofilament strand was then threaded through the lower bearing, after which the lower cap was reclamped in position. The monofilament strand was then pulled downward towards the upper end of the evaporation tube. A second polycaprolactam strand was located on a pirn above and to the side of the upper end of the evaporation tube, as shown in Figure 1. The second strand was a 140 denier, 36 filament yarn. Both strands were obtained from Badische Corporation of Anderson, South Carolina. A strand guide bar was positioned immediately above the upstream end of the evaporation tube and was aligned very close to the path which the monofilament strand would ulti- matety take after completion of stringup. The second strand (the multifilament strand) was passed over the guide, the second strand changing direction of travel by contacting the guide bar. The second prin had an associated balloon guide which positioned the second strand on the guide bar at a point between the guide bar and the point at which the first strand came closest to the guide bar. The guide bar was aligned so close to the path of the first strand that the first strand barely touched the second strand, but the path of the first strand was not substantially deflected nor did the first strand ever touch the guide bar once stringup was complete. Both strands were then directed through a 10 metre long evaporation tube and wound twice around a pair of rollers, as shown in Figure 1. Both rollers had surface speed of 690 metres per minute, with the larger roller having a diameter of about 10 centimetres and the small roller having a diameter of about 2.5 centimetres. The winding of the coherent yarn on a single take-up pirn was then begun as shown in Figure 1.

A conductive mix was made by dispersing 6 parts (by weight) of conductive carbon black into 4 parts of polycaprolactam chip and 90 parts of 70% formic acid. The carbon black particles were obtained from Cabot Corporation of 200 Raritan Centre, Parkway, Edison, N.J. 08817. The carbon black was labelled Vulcan XC-72R. The polycaprolactam chip was obtained from Badische Corporation, Freeport, Texas, the chip being designated as Nylon 6 grade 206 chip.

After the winding of the strands was begun, the valve leading to the mix applicator was opened, filling the reservoir with mix. The stringup procedure must be performed as decribed above because the monofilament strand will completely disintegrate within about 3 seconds if the acid remains substantially unevaporated thereon.

The product yarn of the above described process had intermittent solvent bonds averaging 5 mm to 10 mm apart. If the gap (between the first and second strands) at the guide was widened to as much as 3 mm, the solvent bonds may average one every 200 mm, and the product still shows improved beaming over other prior art supported yarns, such as twisted yarns. The product made from the process described above was a 161 denier 37 filament supported antistatic yarn which had a breaking strength of about 4.4 grams per denier. The breaking strength of both original strands was approximately 4.4 grams per denier. The mix added approximately 1 denier to the sum of the original strand deniers. The product of this example is a "simple side-by-side" supported, solvent-bonded, antistatic yarn, which is the most preferred product of the present invention.

The yarn made by the process of this example was used in the manufacture of Polypropylene Carpet Primary Fabric. The fabric was manufactured by Amoco Fabrics, South Hamilton Street, Dalton, Georgia 30720. The fabric was designated Polybac AS, style number 2605.

## Claims

1. An antistatic yarn comprising at least one conductive strand composed of synthetic plastics material, said conductive strand having finely divided electrically conductive material suffused thereinto and at least one support strand composed of synthetic plastics material characterised in that said conductive strand is intermittently solvent bonded along its length to said at least one support strand.

2. An antistatic yarn as claimed in claim 1, characterised in that said yarn comprises a plurality of support strands, said conductive strand being intermittently bonded along its length to more than one of said support strands.

3. An antistatic yarn as claimed in claim 1, characterised in that said conductive and said support strands are composed of polyamide.

4. An antistatic yarn as claimed in claim 3, characterised in that the polyamide is a polycaprolactam.

5. An antistatic yarn as claimed in any of claims 1 to 4, characterised in that said finely divided electrically conductive material is carbon black.

6. An antistatic yarn as claimed in any of claims 1 to 5, in which the conductive strands and support strands are continuous filaments.

7. A carpet comprising an antistatic yarn as claimed in any of claims 1 to 6.

8. A carpet as claimed in claim 7, characterised in that it is comprised of a composite yarn composed of an antistatic yarn as claimed in any of claims 1 to 6 interlaced into a carpet yarn.

9. A carpet as claimed in claim 8, characterised in that the carpet yarn is a continuous filament yarn.

10. A carpet as claimed in claim 8 or 9, characterised in that the carpet yarn is composed of polyamide.

11. A method of producing an antistatic yarn which comprises suffusing a finely divided electrically conductive material into a strand composed of a synthetic plastics material to form a conductive strand by applying to the travelling strand a dispersion of said finely divided material in a liquid which is a solvent for synthetic plastics material of both the strand which is to become the conductive strand and the support strands, but does not dissolve or react with the said finely divided material, characterised in that the support strand or strands are brought into generally side-by-side relationship with the potentially conductive strand before a substantial amount of the solvent carried by the potentially conductive strand has evaporated therefrom and allowing said potentially conductive strand to contact said support strand or strands at intermittent points along the length thereof, the potentially conductive strand being allowed to contact only the support strand or strands and the atmosphere until the liquid has substantially evaporated from the potentially conductive strand and in that the evaporation of liquid being effected by passing the potentially conductive strand and the support strand or strands in generally side-by-side relationship and in contact at intermittent points along their length through an evaporation zone maintained at an elevated temperature whereby to effect intermittent solvent bonding of the conductive strand to the support strand or strands along the length thereof.

12. A method as claimed in claim 11, characterised in that the synthetic plastics material is polyamide.

13. A method as claimed in claim 12, characterised in that the polyamide is a polycaprolactam.

14. A method as claimed in claim 11, characterised in that air at an elevated temperature is passed through the evaporation zone in countercurrent to the direction of travel of the potentially conductive and support strands.

15. A method as claimed in any of claims 11 to 14, in which the strands are continuous filaments.

16. A method as claimed in any of claims 11 to 15, characterized in that when the potentially conductive strand and support strand or strands are brought into generally side-by-side relationship the distance between them is no greater than 3 mm and the path of travel of the potentially conductive strand is substantially undeflected.

17. A method as claimed in any of claims 11 to 16, characterized by the solvent being formic acid.

## Patentansprüche

1. Antistatisches Garn mit mindestens einem leitenden Strang aus Kunststoffmaterial, der fein verteiltes elektrich leitendes Material in ihn eingebracht aufweist, sowie mit mindestens einem Tragstrang aus Kunststoffmaterial, dadurch gekennzeichnet, daß der leitende Strang absatzweise längs seiner Länge mit den mindestens einen Tragstrang lösungsmittelverklebt ist.

2. Antistatiches Garn nach Anspuch 1, dadurch gekennzeichnet, daß das Garn eine Vielzahl von Tragsträngen aufweist und der leitende Strang absatzweise längs seiner Länge mit mehr als einem der Tragstränge verklebt ist.

3. Antistatisches Garn nach Anspruch 1, dadurch gekennzeichnet, daß der leitende Strang und der Tragstrang aus Polyamid bestehen.

4. Antistatisches Garn nach Anspruch 3, dadurch gekennzeichnet, daß das Polyamid ein Polycaprolactam ist.

5. Antistatisches Garn nach einem der Ansprüche 1 bis 4, dadurch gekennzeichnet, daß das fein verteilte elektrisch leitende Material Ruß ist.

6. Antistatisches Garn nach einem der Ansprüche 1 bis 5, bei dem die leitenden Stränge und Tragstränge kontinuierliche Fäden sind.

7. Teppich mit einem antistatischen Garn nach einem der Ansprüche 1 bis 6.

8. Teppich nach Anspruch 7, dadurch gekennzeichnet, daß der ein zusammengesetztes Garn aufweist, das aus einem mit einem Teppichgarn verflochtenen antistatichen Garn nach einem der Ansprüche 1 bis 6 besteht.

9. Teppich nach Anspruch 8, dadurch gekenn= zeichnet, daß das Teppichgarn ein kontinuierliches Fadengarn ist.

10. Teppich nach Anspruch 8 oder 9, dadurch, gekennzeichnet, daß das Teppichgarn aus Polyamid besteht.

11. Verfahren zum Herstellen eine antistatischen Garns, bei dem ein fein verteiltes elektrisch leitendes Material in einem aus einem Kunststoffmaterial bestehenden Strang zur Bildung eines leitenden Stranges dadurch eingebracht wird, daß auf den sich bewegenden Strang eine Dispersion des fein verteilten Materials in einer Flüssigkeit aufgebracht wird, die in Lösungsmittel für das Kunststoffmaterial sowohl des Stranges, der der leitende Strang werden soll, als auch des Trangstrangs ist, jedoch das fein verteilte Material nicht auflöst oder mit diesem reagiert, dadurch gekennzeichnet, daß der Tragstrang bzw. die Tragstränge und der potentiell leitende Strang etwa nebeneinanderliegend angeordnet werden, bevor eine wesentliche Menge des von dem potentiell leitenden Stranges getragenen Lösungsmittels von diesem verdampft ist, daß es ermöglicht wird, daß der potentiell leitende Strang den Tragstrang bzw. die Tragstränge an absatzweisen Punkten längs ihrer Länge berührt, daß es ermöglicht wird, daß der potentiell leitende Strang nur den Tragstrang bze. die Tragstränge und die Atmosphäre berührt, bis die Flüssigkeit von dem potentiell leitenden Strang im wesentlichen verdampft ist, und daß die Verdampfung der Flüssigkeit dadurch bewirkt wird, daß der potentiell leitende Strang und der Tragstrang bzw. die Tragstränge etwa nebeneinanderliegend angeordnet und in Kontakt an absatzweisen Punkten längs ihrer Länge durch eine Verdampfungszone geführt werden, die bei erhöhter Temperatur gehalten wird, wodurch ein absatzweises Lösungsmittelverkleben des leitenden Stranges mit dem Tragstrang bzw. den Tragsträngen längs ihrer Länge bewirkt wird.

12. Verfahren nach Anspruch 11, dadurch gekennzeichnet, daß das Kunststoffmaterial ein Polyamid ist.

13. Verfahren nach Anspruch 12, dadurch gekennzeichnet, daß das Polyamid ein Polycaprolactam ist.

14. Verfahren nach Anspruch 11, dadurch gekennzeichnet, daß Luft mit erhöhter Temperatur durch die Verdampfungszone in Gegenströmung zu der Bewegungsrichtung des potentiell leitenden und des Tragstrangs geführt wird.

15. Verfahren nach einem der Ansprüche 11 bis 14, bei dem die Stränge kontinuierliche Fäden sind.

16. Verfahren nach einem der Ansprüche 11 bis 15, dadurch gekennzeichnet, daß, wenn der potentiell leitfähige Strang und der Tragstrang bzw. die Tragstränge etwa nebeneinanderliegend angeordnet werden, der Abstand zwischen ihnen nicht größer als 3 mm und der Bewegungsweg des potentiell leitenden Stranges im wesentlichen unabgelenkt ist.

17. Verfahren nach einem der Ansprüche 11 bis 16, dadurch gekennzeichnet, daß das Lösungsmittel Ameisensäure ist.

## Revendications

1. Fil antistatique comportant au moins un brin conducteur constitué de matière plastique synthétique, ledit brin conducteur ayant une matière électriquement conductrice finement divisée et diffusée à l'intérieur et au moins un brin de soutien constitué de matière plastique synthétique, caractérisé en ce que ledit brin conducteur est lié par solvant, par intermittence suivant sa longueur, avec ledit brin de soutien.

2. Fil antistatique selon la revendication 1, caractérisé en ce que ledit fil comporte plusieurs brins de soutien, ledit brin conducteur étant lié par intermittence suivant sa longueur avec plus d'un desdits brins de soutien.

3. Fil antistatique selon la revendication 1, caractérisé en ce que ledits brins conducteurs et desdits brins de soutien sont constitués de polyamide.

4. Fil antistatique selon la revendication 3, caractérisé en ce que le polyamide est un poly- caprolactame.

5. Fil antistatique selon l'une quelconque des revendications 1 à 4, caractérisé en ce que ladite matière électriquement conductrice finement divisée est du noir de carbone.

6. Fil antistatique selon l'une quelconque des revendications 1 à 5, dans lequel les brins conducteurs et les brins de soutien sont des filaments continus.

7. Tapis comportant un fil antistatique selon l'une quelconque des revendications 1 à 6.

8. Tapis selon la revendication 7, caractérisé en ce qu'il est constitué d'un fil composite composé d'un fil antistatique selon l'une quelconque des revendications 1 à 6, entrelacé dans un fil de tapis.

9. Tapis selon la revendication 8, caractérisé en ce que le fil de tapis est un fil en filaments continus.

10. Tapis selon la revendication 8 ou 9, caractérisé en ce que le fil de tapis est constitué en polyamide.

11. Procédé pour fabriquer un fil antistatique, qui comporte la diffusion d'une matière électriquement conductrice finement divisée dans un brin constitué de matière plastique synthétique pour former un bring conducteur en appliquant au brin en déplacement une dispersion de ladite matière finement divisée dans un liquide qui soit un solvant de la matière plastique synthétique du brin qui doit devenir le brin conducteur ainsi que des brins de soutien, mais qui ne dissolve pas ladite manière finement divisée et ne réagisse pas avec elle, caractérisé en ce que le brin our les brins de soutien sont amenés sensiblement en position côte à côte par rapport au brin potentiellement conducteur avant qu'une quantité importante de solvant porté par le brin potentiellement conducteur se soit évaporée de ce brin et on laisse ledit brin potentiellement conducteur venir en contact avec ledit brin ou lesdits brins de soutien en des points espacés sur leur longueur, en ne laissant le brin potentiellement conducteur ne venir en contact qu'avec le brin ou les brins de soutien et l'atmosphère jusqu'à ce que le liquide se soit notablement évaporé du brin potentiellement conducteur et en ce que l'évaporation du liquide est effectuée en faisant passer le brin potentiellement conducteur et le brin ou les brins de soutien en position sensiblement côte à côte et en contact en des points espacés sur leur longueur dans une zone d'évaporation maintenue à une température élevée afin d'effectuer par intermittence une liaison par solvant entre le brin conducteur et le brin ou les brins de soutien sur leur longueur.

12. Procède selon la revendication 11, caractérisé en ce que la matière plastique synthétique est un polyamide.

13. Procédé selon la revendication 12, caractérise en ce que le polyamide est un polycapro- lactame.

14. Procédé selon la revendication 11, caractérisé en ce qu'on fait passer de l'air à température élevée dans la zone d'évaporation à contre- courant par rapport au sens de déplacement des brins potentiellement conducteur et de soutien.

15. Procédé selon l'une quelconque des revendications 11 à 14, dans lequel les brins sont des filaments continus.

16. Procédé selon l'une quelconque des revendications 11 à 15, caractérisé en ce que le brin potentiellement conducteur et le brin ou les brins de soutien sont amenés en position sensiblement côte à côte, la distance entre eux n'est pas supérieure à 3 mm et le parcours de déplacement du brin potentiellement conducteur n'est pas sensiblement dévié.

17. Procédé selon l'une quelconque des revendications 11 à 16, caractérisé en ce que le solvant est l'acide formique.
